

1

2,895,785

## NEW COLOURATION PROCESS FOR TEXTILE MATERIALS

Frederick Richard Alsberg and Arthur Hutchinson Wyld, Manchester, England, assignors to Imperial Chemical Industries Limited, London, England, a corporation of Great Britain

No Drawing. Application March 31, 1958  
Serial No. 724,850

Claims priority, application Great Britain April 10, 1957

3 Claims. (Cl. 8—65)

The invention relates to a new colouration process for 15 textile materials and more particularly to a new colouration process for producing patterned effects on textile materials by resist printing.

It is known that white resist patterns can be obtained on cellulosic textile materials by printing the textile materials with a resist paste containing sodium formaldehyde sulphoxylate and dimethylphenylbenzylammonium chloride, drying, and then padding the textile materials with a solution of a reactive dyestuff, for example an azo or anthraquinone dyestuff containing a dichloro-triazinyl radical, and finally heating to fix the dyestuff. This process has the disadvantage that the resist paste is unstable when it is exposed to atmospheric oxidation, the outlines of the resisted portions are not always well-defined, and slight discolouration of the ground shade is sometimes produced. Furthermore when a coloured resist using a vat dyestuff is printed alongside a white resist, the colour yield from the vat dyestuff is appreciably reduced where the vat dyestuff paste comes into contact with the white resist paste.

We have now found that organic amino compounds can be used to give effective resists under reactive dyestuffs and that the disadvantages of the known resist printing process can be avoided by using resist pastes containing organic amino compounds.

According to our invention we provide a new colouration process for textile materials which comprises locally applying to the textile materials a resist paste comprising an organic amino compound and a thickening agent, and subsequently padding the textile materials with a solution of a reactive dyestuff as hereinafter defined, and when the textile material is of natural or regenerated cellulose, an alkaline compound or a compound which on heating or steaming gives rise to an alkaline compound.

By a "reactive dyestuff" we mean a dyestuff containing a reactive halogen atom or other reactive atom or group, that is to say a halogen atom or other group capable of reacting with the fibre. Usually, reactive dyestuffs are water-soluble. They are principally used for vegetable fibres and regenerated cellulose, also using an alkali treatment to cause reaction therewith, and preferably have a small affinity for these materials when applied under conditions other than those giving rise to reaction with the material, so that unreacted dyestuff may readily be washed from the material after the colouration process. Examples of classes of such reactive dyestuffs include dyestuffs containing a s-triazinyl radical carrying one or two chlorine or bromine atoms directly attached to the triazine ring, dyestuffs containing a pyrimidyl radical carrying one or two chlorine or bromine atoms directly attached to the pyrimidine ring, and dyestuffs containing a beta - halogenopropionyl, beta - halogenoethylsulphonyl, beta - halogenoethylsulphamyl, beta-sulphatoethylsulphonyl, beta-hydroxyethylsulphonyl, chloroacetylarnino, beta - (chloromethyl)-beta-sulphatoethylsulphamyl, alkyl phosphite, or sulphon fluoride radi-

2

cal. The dyestuffs in these classes may be for example nitro dyestuffs or dyestuffs of the azo, anthraquinone or phthalocyanine series and may be metal free or may contain metal in complex formation. Specific examples

5 of suitable dyestuffs are described in United Kingdom specification No. 209,723 in Examples 1 and 2, United Kingdom specification No. 298,484 in Example 1, in United Kingdom specification Nos. 460,224, 733,471, 740,533, 775,308, 772,030, 774,925, 780,591, 781,930, 10 785,120, 785,222 and in German Auslegeschrift No. 1,008,313.

The organic amino compounds should preferably be soluble in water. They may contain substituted or unsubstituted amino groups and may be for example mono-amines such as diethylamine, diamines such as ethylene diamine, polyamines such as diethylene triamine, triethylene tetramine, tetraethylene pentamine, acid amides such as formamide or dimethylformamide, amino-alcohols such as mono-, di-, and tri-ethanolamine and beta-diethyl-20 aminoethanol and cyclic amino compounds such as hexamethylene tetramine and polyvinylpyrrolidone. It is preferred however to use as the amino compound, an amino-acid for example glycine, benzylglycine, phenylglycine, phenylglycine-o-carboxylic acid, methyltaurine, N-methyl-, N-ethyl- and N-benzylanthranilic acid, N-benzylsulphoanthranilic acid, 2-ethylamino-5-sulphobenzoic acid and especially, sarcosine. The amino-acid may be used in the form of a water-soluble salt, for example an alkali metal salt.

25 30 The quantity of organic amino compound required will depend on the nature of the organic amino compound used and also on the thickening agent and dyestuff used but in general it is found that between 2% and 10% of organic amino compound calculated on the weight of the resist paste gives satisfactory results in practice. Quantities outside these limits may be used if desired, provided that there is a molecular excess of the amino compound, preferably at least 5 molecular proportions, relative to the amount of dyestuff present.

35 40 As a suitable thickening agent for use in the resist paste there may be mentioned, for example, British gum thickening.

The textile materials which may be coloured by the process of our invention include not only cellulosic materials such as cotton and viscose but also protein materials such as silk and wool and textile materials made from artificial fibres such as nylon.

45 50 The resist paste may be prepared by mixing the thickening agent with the organic amino compound, preferably in aqueous solution, and the paste may be applied to the textile material by, for example, stencil, block, screen or machine printing processes. If desired other resists, for example vat dyestuff coloured resists, may also be applied. The dyestuff solution may then be applied 55 by padding. The alkaline compound for example sodium carbonate or the compound which on heating or steaming gives rise to an alkaline compound, for example sodium bicarbonate, is conveniently added to the dyestuff solution but, if desired, it may be applied to the textile material before or after padding with the dyestuff solution. After application of the dyestuff solution and the alkaline compound, or compound which on heating or steaming gives rise to an alkaline compound, the textile material may be steamed, or heated for example in a hot air chamber or on steam-heated drying cylinders to fix the dyestuff. The textile material may then be rinsed in cold water and finally treated in a hot dilute aqueous solution of a detergent, for example, a sulphated fatty alcohol or a condensation product of alkylphenols with ethylene oxide, and finally rinsed in water and dried.

60 65 70 75 80 By the process of the invention good clear white resists with sharp outlines are obtained and there is no appreci-

able reduction in the colour yield of vat dyestuffs which come into contact with the resist paste containing the organic amino compound.

The invention is illustrated but not limited by the following examples in which the parts are by weight.

*Example 1*

Cotton cloth is printed with a resist paste made up by mixing together 70 parts of British gum thickening and 30 parts of a 13.4% aqueous solution of the sodium salt of sarcosine. The cloth is dried and then padded through a dyestuff solution prepared by dissolving 2 parts of the dyestuff described in Example 3 of Belgian specification No. 543,214 in 87 parts of water and adding 10 parts of 5% sodium alginate thickening and then 1 part of sodium bicarbonate. The cloth is dried in a hot flue and steamed for 5 minutes in a conventional ager, rinsed well in cold water and then treated for 5 minutes in a bath containing 1 part of a detergent mixture, consisting of alkylphenols condensed with ethylene oxide and a sulphated fatty alcohol, in 1000 parts water at between 85° and 100° C. The cloth is finally rinsed in cold water and dried.

The portions printed with the resist paste prevent the fixation of the dyestuff and a good clear white pattern on a brilliant red background is obtained.

In the above example, instead of fixing the dyestuff on the padded cloth by drying and then steaming, the dyestuff may be fixed by passing the cloth over steam-heated cylinders or by heating in a hot air dryer.

In place of the 2 parts of dyestuff used in the above example, there may be used 2 parts of the dyestuff described in Example 1 of Belgian specification No. 543,215 or 2 parts of the dyestuff described in Example 1 of Belgian specification No. 543,216 when a white pattern on a yellow ground and a white pattern on a blue ground respectively are obtained.

*Example 2*

In place of the resist paste used in Example 1, there may be used a resist paste made by mixing together 70 parts of British gum thickening, 15 parts of a 13.4% aqueous solution of the sodium salt of sarcosine and 15 parts of a 50% aqueous paste of zinc oxide. A white resist is obtained.

In place of the 15 parts of 50% aqueous paste of zinc oxide used in the above example there may be used 15 parts of a 50% aqueous paste of titanium dioxide.

*Example 3*

In place of the resist paste used in Example 1 there may be used resist paste made up by mixing together 70 parts of British gum thickening, 5 parts of 2-ethylamino-5-sulphobenzoic acid and 25 parts of water when a similar result is obtained.

*Example 4*

In place of the resist paste used in Example 1 there may be used a resist paste made up by mixing 70 parts of British gum thickening, 10 parts of hexamethylenetetramine and 20 parts of water when a similar result is obtained.

*Example 5*

A cloth made from polyamide fibre is printed with a resist paste made up by mixing 70 parts of British gum thickening and 30 parts of a 13.4% aqueous solution of the sodium salt of sarcosine. The printed cloth is dried and padded in a dyestuff solution made up by dissolving 0.5 part of the dyestuff described in Example 1 of Belgian specification No. 543,214, 3 parts of urea, 1 part of ammonium oxalate and 10 parts of a 5% sodium alginate thickening in 85.5 parts of water.

The cloth is dried on steam heated drying cylinders, steamed for 5 minutes in a conventional steamer, rinsed well in cold water and then treated for 5 minutes at 85° C. in a solution of 2 parts of a detergent mixture, consisting of alkylphenols condensed with ethylene oxide and a

sulphated fatty alcohol, and 2 parts of soda ash in 1000 parts of water. The cloth is rinsed in cold water and dried.

The portions printed with the resist paste prevent the fixation of dyestuff and a good clear white pattern on a brilliant red background is obtained.

*Example 6*

Cloth made from natural silk is printed with a resist paste prepared as described in Example 5. The cloth is dried and padded with a dyestuff solution made by dissolving 0.5 part of the dyestuff described in Example 1 of Belgian specification No. 543,215 in 88.5 parts of water and adding 10 parts of 5% sodium alginate thickening and 1 part of sodium bicarbonate. The fabric is dried in a hot air chamber, steamed for 5 minutes, rinsed well in cold water and then treated for 5 minutes at 40° C. in a solution of 2 parts of the detergent mixture used in Example 1 in 1000 parts of water. The cloth is rinsed in cold water, and dried.

The portions printed with the resist paste prevent the fixation of dyestuff and a good clear white pattern on a blue background is obtained.

*Example 7*

In place of the dyestuff solution used in Example 1 there is used a dyestuff solution made by dissolving 1 part of the blue disazo dyestuff shown in the first formula on page 586 of "The Chemistry of Synthetic Dyes," volume 1, by K. Venkataraman (New York Academic Press, 1952), and 5 parts of urea in 83 parts of water and adding 10 parts of 5% sodium alginate thickening and 1 part of sodium bicarbonate.

The areas printed with the resist paste prevent the fixation of dyestuff and a good clear white pattern is produced on a greenish-blue ground.

*Example 8*

In place of the dyestuff solution used in Example 1 there is used a dyestuff solution made by dissolving 0.5 part of the dyestuff prepared as described below and 10 parts of urea in 79.5 parts of water and adding 10 parts of a 5% sodium alginate thickening and 1 part of sodium bicarbonate. The fixation of the dyestuff is carried out by the steaming process.

The areas printed with the resist paste prevent the fixation of the dyestuff and a white patterned effect is produced on a turquoise blue ground.

The dyestuff used in this example may be made by treating 50 parts of the sodium salt of copper phthalocyaninetetra-4-sulphonic acid with 475 parts of chlorosulphonic acid at 115° C. for 4 hours, pouring the mixture onto ice and treating the precipitated sulphonchloride with a solution of 12.8 parts of 2-chloroethylamine hydrochloride in aqueous sodium bicarbonate when the sulphonchloride groups are in part replaced by sulphon-β-chloroethylamide groups and in part hydrolysed to sulphon acid groups.

*Example 9*

In place of the 30 parts of a 13.4% aqueous solution of the sodium salt of sarcosine used in Example 1 there may be used 30 parts of 16.7% solution of diethylamine, ethylene diamine, benzylglycine, N-ethylanthranilic acid, 2-ethylamino-5-sulphobenzoic acid, N-methylglucosamine, or polyvinylpyrrolidone or a 33% solution of hexamethylenetetramine or tetraethylene pentamine or a 7% solution of glycine or methyltaurine when similar results are obtained.

*Example 10*

Cotton cloth is machine printed with a copper roller using a resist paste made up by mixing together 70 parts of British gum thickening and 30 parts of a 13.4% aqueous solution of the sodium salt of sarcosine. The cloth is then printed in a different pattern with a second

copper roller using a vat printing paste made up by mixing 6 parts of Caledon Printing Jade Green XBN (the dyestuff C.I. Vat Green 1 of the "Colour Index," 1957 edition, volume II), 75 parts British gum thickening, 6 parts of sodium carbonate, 5 parts of glycerol, 8 parts of sodium formaldehyde sulphonylate.

The cloth is then dried and padded through the dyestuff solution used in Example 1, steamed for 5 minutes, rinsed in cold water, treated for 2 minutes in a cold aqueous solution containing 0.2% sodium dichromate

5 and 0.2% acetic acid, rinsed again and treated for 5 minutes in a boiling aqueous solution containing 0.3% of the detergent mixture used in Example 1, rinsed in cold water, and finally dried. White and green patterned effects on a brilliant red background are obtained.

The following table describes in the first column further examples of dyestuffs which may be substituted in Example 1 for the dyestuff used therein; in each case there is obtained a good clear white pattern on a background of the colour indicated in the second column.

| Dyestuff | Colour           |
|----------|------------------|
|          | Greenish-yellow. |
|          | Reddish-yellow.  |
|          | Yellow.          |
|          | Bluish-red       |
|          | Do.              |
|          | Do.              |
|          | Greenish-blue.   |

| Dyestuff | Colour          |
|----------|-----------------|
|          | Reddish blue.   |
|          | Greenish-blue.  |
|          | Turquoise-blue. |

The dyestuff obtained by treating 115 parts of copper pythalocyanine with 1,200 parts of chlorosulphonic acid at 138° C. for 4 hours, pouring the mixture on to ice and treating the precipitated sulphonchloride with a solution of 60 parts of 3-chloro-2-hydroxypropyl-amine hydrochloride in aqueous sodium bicarbonate, when the sulphonchloride groups are in part replaced by 3-chloro-2-hydroxypropylsulphamyl groups and in part by sulphonic acid groups.

## What we claim is:

1. New colouration process for textile materials, selected from the group consisting of cotton, viscose, silk, wool, and nylon, which comprises locally applying to the textile materials a resist paste comprising an organic amino compound, selected from the group consisting of amino acids, amino alcohols, saturated cyclic amines, and aliphatic mono- and polyamines, and a thickening agent, and subsequently padding the textile materials with a solution of a reactive dyestuff having a reactive group capable of reacting with the fiber, and, when the textile material is of cellulose, a member selected from the group consisting of an alkaline compound and a com-

30 pound which on being subjected to an elevated temperature gives rise to an alkaline compound.

2. Process as claimed in claim 1 wherein the organic amino compound used is sarcosine.

3. Process as claimed in claim 1 wherein the resist paste contains between 2% and 10% by weight of the organic amino compound.

## References Cited in the file of this patent

## UNITED STATES PATENTS

40 1,913,410 Rivat \_\_\_\_\_ June 13, 1933  
2,726,133 Helfenberger \_\_\_\_\_ Dec. 6, 1955